

Jan. 19, 1932.

L. P. F. VAN DER GRINTEN ET AL 1,841,653

PROCESS FOR DEVELOPING POSITIVE DIAZO PRINTS

Filed Aug. 11, 1928



Inventors:

L. P. F. van der Grinten and

K. J. J. van der Grinten

By Emil Bönnelycke  
Attorney

## UNITED STATES PATENT OFFICE

LODEWIJK PIETER FRANS VAN DER GRINTEN AND KAREL JAN JOSEF VAN DER GRINTEN,  
OF VENLO, NETHERLANDS, ASSIGNORS TO FRANS VAN DER GRINTEN, OF VENLO,  
LIMBURG, NETHERLANDS

## PROCESS FOR DEVELOPING POSITIVE DIAZO PRINTS

Application filed August 11, 1928, Serial No. 299,042, and in the Netherlands August 22, 1927.

It is common knowledge that the positive diazo printing process is based on two properties of the diazo compounds:

- (a) Their sensitiveness to light. The diazo compounds are decomposed (probably and on the whole into phenols) by exposure to light;  
(b) Their property of forming azo dyes with substances known as azo-dye components.

Reaction (b) takes place mostly with the co-operation of alkalis. In the photographic diazo printing process, a film containing a diazo compound and generally disposed on paper is exposed to light under a transparent image, drawing or tracing, so that the diazo compound is decomposed on those areas of the film which are reached by light.

An azo dye is formed in the areas which are unaffected by light (and in which the diazo compound has remained unaltered) by treating the exposed film with an azo-dye component and alkali, while the areas which have been exposed to light remain colourless when treated in this manner. The image is simultaneously fixed, because after being subjected to this treatment (which may be also considered as a developing treatment) the image-forming areas (now containing a dye) as well as the background reached by light, are stable under any further action thereof. The positive diazo-printing process does not involve a separate fixing operation, which is necessary in most of the other photographic processes and which usually consists in removing either non-decomposed light-sensitive initial materials or certain substances formed by the action of light. In the positive photographic diazo printing process, the developing operation (which is simultaneously a fixing operation) consists exclusively in an addition of substances. It is in fact sufficient to add an alkali for developing purposes when the azo-dye components are initially embodied in the light-sensitive film, this being made possible in practice by using certain diazo compounds such as for example diazo anhydrides. The simplest known manner in which the alkali may be added is to subject the exposed sensitive film to the action of gaseous

ammonia, the prints being disposed in a developing tank containing ammonia vapour. The advantage of this method of proceeding is that developing baths are dispensed with, so that the pictures thus developed need not be dried.

This developing method has however the following disadvantages:

(a) The developing operation is comparatively lengthy, especially in the winter. At low temperature, the prints must remain in the ammonia-charged atmosphere for half an hour or more in order to be fully developed.

(b) When no complicated mechanical apparatus is used, this developing operation is highly tedious because of the unpleasant and injurious alkaline vapours.

The developing tanks must therefore be often in the open and the prints developed smell of ammonia for a long time.

These two main disadvantages are the reason why the diazo printing process with what is known as dry development is not used in practice as widely as the simplicity of the process might have warranted.

The above disadvantages are not to be found in the method of developing diazo prints in baths (described for example in Eder's "Handbuch der Photographie", 1899, pages 563-565, and in "Photographische Korrespondenz", 1895, pages 284-285) because (a) the print may be developed in a few seconds, and (b) non-volatile alkalis may be used which evolve no offensive and injurious vapours.

This method however lacks the characteristic advantages inherent in dry development with the aid of vapours. Moreover, a difficulty involved in the use of baths is that the always more or less soluble azo-dyes merge one into the other, with the result that the images obtained are not sharp and the clearness of the background is affected.

The present process has the advantages of both the methods described in the foregoing while their disadvantages are entirely avoided. According to the present invention, an extremely thin layer of an alkaline liquid (which if necessary may contain an azo-dye component) is uniformly spread over the

whole area to be developed. Friction may be avoided, in which case the procedure consists in applying an extremely thin layer of the developing liquid on the surface to be 5 developed. This makes it possible:

- (a) To develop in a few seconds;
- (b) To avoid offensive vapours by using non-volatile alkalis;
- (c) To use a very thin layer of liquid, so 10 that the prints remain dry and the colours do not merge;
- (d) To use diazo compounds (by applying the alkaline developer together with the azo-dye components) which cannot be used (or 15 can be used only under certain conditions) together with azo-dye components in the light-sensitive film, whereby the selection of diazo compounds is very large.

In the accompanying drawing, the single 20 figure is a side view, partly in vertical section, of an apparatus for applying the developer.

This apparatus, which is of extremely simple character, comprises two vertically superposed and rubber-covered rolls *a* and *b*, the lower roll *b* revolving in a trough *c* containing the developing liquid and the upper roll bearing on the lower one by gravity or being 25 pressed (hard when necessary) thereon by suitable means such as for example screws 30 (*c*) acting upon the bearings of the roll. The lower roll is driven while the upper roll is preferably moved at the same peripheral velocity so that there is no friction at the line 35 of contact.

The lower rubber roll *b* collects, while rotating, developing liquid from the trough *c* and conveys it to the line of contact of the two rolls. Here the liquid is practically entirely retained and flows back uniformly.

This extremely simple apparatus comprises moreover a small table *d* disposed in front of the upper roll and fitted with a simple guiding and flattening device *s* to prevent 45 creases from being formed. A stripper may be advantageously provided to prevent the paper from adhering to the rolls. This stripper may be constituted by blades *f* projecting as far as the grooves *g* of the rolls.

50 When a print is passed between the two rolls with the side to be developed facing downwards, the said side is wetted by the developing liquid for a very short instant and is pressed between the two rubber rolls immediately after. To this end, the print *h* is laid on the table *d* with the image side upwards and is pushed between the upper roll *a* and the flattening device *s*; the roll *a* picks up the print and conveys it through the rolls 55 *a* and *b*.

The print comes out at the other side between the rolls; it carries a sufficient quantity of developer and is practically dry. The chemical development reaction now takes 60 place within a very short time (a few minutes

at most) in the film thus treated. There is however no necessity to wait, because the print develops of itself without further supervision.

Four metres of prints may be easily developed per minute when the width is suitable (usually 100 cm.). This rate of operation may be considerably increased by using a very concentrated developing liquid; it is also possible however, to work, if required, 75 at a slower rate by using more dilute developers.

For small installations this simple apparatus may be replaced by smaller, simpler and cheaper means with the aid of which it 80 is likewise possible to provide the light print with a uniform thin layer of developing liquid.

The developers which may be used according to this invention are aqueous solutions of alkalis or alkaline-reacting substances, mixed if necessary with azo-dye components such as phloroglucinol, resorcinol, resorcinic acids, naphthols, phenols, naphthol-sulphonic acids and the like. Should the light-sensitive film 90 be devoid of substances preventing the prints from turning yellow, such substances may also be added to the developer.

The substances which prevent the prints from turning yellow may be incorporated in 95 the light-sensitive film as well as in the developing liquid. As a general rule, reducing substances which are stable in an acid medium are preferably used in the light-sensitive film and those which are stable in 100 an alkali medium are used in the developing liquid.

The alkaline substances used may advantageously be potassium carbonate, sodium carbonate and ammonium carbonate (the latter not so much to be recommended because it has a smell of ammonia) preferably mixed with buffer salts such as secondary phosphates, secondary citrates and generally salts of polyvalent weak acids and the like.

105 Buffer salts are salts by which the intensity of the alkaline reaction is decreased without affecting the potential alkaline reaction, especially salts of polyvalent acids, such as phosphoric acid, citric acid and the like, and salts having a neutral reaction, such as secondary sodium phosphate; which salt, for instance, if added to an alkali solution, forms tertiary phosphate. Said salt has an alkaline reaction, but in the presence of an excess of secondary salt the concentration of the OH-ions, which causes the intensity of the alkaline reaction, is very considerably decreased with respect to the original alkali solution and yet its alkaline action (capacity 110 of neutralizing acids) remains the same.

In order that the printing may be as uniform as possible, a wetting agent such as alcohol, glycerine, Turkey-red oil and the like may be added to the developing liquid.

*Example 1.*—Prints obtained by exposing diazo-printing paper the light-sensitive film of which contains 1.dimethylamino.2.chlorobenzene.4.diazonium chloride, or 4.diethyl-5 amino-benzol-diazonium chloride, are printed with a developer by being guided between the rubber-covered rolls described in the foregoing. The said developer is an aqueous solution of 20 parts by weight of potassium carbonate, 30 parts by weight of disodium phosphate and 1.2 parts by weight of phloroglucinol, so that the print is developed. Positive images are thus obtained in dark to black colour on a light background. 10 In the developer, the 1.2 parts by weight of phloroglucinol may be replaced by 4 parts by weight of resorcinol, 5 parts by weight of  $\beta$ -naphthol, 5 parts by weight of  $\beta$ -oxy-naphthoic acid anilide, 3 parts by weight of 2.7.20 oxynaphthaline and the like. These are then dissolved in quantities of soda lye sufficient for dissolution and yield images in various dark colours.

In a similar manner, the potassium carbonate may be replaced by sodium carbonate or ammonium carbonate while disodium phosphate may be replaced by disodium citrate or the like.

The following may be added to the developer to prevent the print from turning yellow: 0.4% of formalin or 1% of urotropin and the like; or 5% of glucose, 2% of sodium lactate, 0.1% of pyrogallol.

The uniform spreading of the developer on the paper is assisted with 5% of methylated alcohol or 3% of glycerine or 1% of Turkey-red oil and the like.

*Example 2.*—A solution is made, which contains 1.8% of 1.diethyl-aminobenzol.4.diazonium chlorostannate and 1% of potassium sulphate. The solution is spread on paper and the like, and dried. After exposure under a drawing of transparent paper, a thin layer of an aqueous solution of 5% of potassium carbonate, 0.5% of phloroglucinol, 0.5% of resorcinol, 10% of potassium chloride, 10% of sodium citrate, 10% sodium hyposulphite and 10% of glucose is uniformly spread over the whole surface of the print with the apparatus shown. An entirely black picture is obtained, which is very stable against any tendency to become yellow, which would not be the case without the reducing means (citrate, hyposulphite and glucose).

*Example 3.*—A thin layer of a developing liquid constituted by an aqueous solution of 40 parts by weight of potassium carbonate and 60 parts by weight of disodium phosphate is spread as in Example 1 on prints obtained by exposing diazo printing papers containing 1.5 parts by weight of 2.7.dioxy-naphthaline and 3% of oxalic acid to 5 parts by weight of 1.dimethylamino.3.5.xylol.4.diazonium chlorostannate; or 0.5 parts by weight of phloroglucinol and 3% of oxalic

acid, or 1.5 parts by weight of triketohexamethylenetrioxym, 0.3 parts by weight of hydroxylamine chloride and 2 parts by weight of tartaric acid to 5 parts by weight of 1.dimethylamino.3.5.xylol.4.diazonium chlorostannate; or the hydroxylamine compound of 0.2 parts by weight of phloroglucinol and two parts by weight of tartaric acid to 1.5 parts by weight of dimethylamino-benzene.4.diazonium chlorostannate; or combinations of these examples. All methods of printing described in Example 1 are also applicable to the present example. 70 75

*Example 4.*—Prints obtained by exposing diazo print papers made of diazo anhydrides with azo dye components are printed as in Examples 1, 2 or 3 and treated with a developer as in Example 3. All methods of printing described in Example 1 are applicable to this example. 80 85

What we claim is:—

1. The process for developing direct positive diazo prints which consists in impressing upon the surface to be developed an alkaline liquid containing an azo-dyestuff component and a reducing agent non-decomposable by alkali, in the form of a uniformly thin film. 90

2. The process for developing direct positive diazo prints which consists in impressing upon the surface to be developed an alkaline liquid containing an azo-dyestuff component and a buffer salt, in the form of a uniformly thin film. 95

3. The process for developing direct positive diazo prints which consists in impressing an alkaline liquid containing an azo-dyestuff component in the form of a uniformly thin film upon an exposed surface having a diazo compound therein, said film containing the azo-dyestuff component in an amount not substantially in excess of that required to couple with the diazo compound. 105

4. The process for developing direct positive diazo prints which consists in saturating throughout its entire area the exposed surface of said prints with a developing liquid containing a non-volatile alkaline substance by spreading said liquid on said surface in the form of a uniformly thin film, the quantity of the developing liquid contained in the film being substantially corresponding to that required to effect development of said surface. 110 115

5. The process for developing direct positive diazo prints which consists in saturating throughout its entire area the exposed surface of said prints with a developing liquid containing a non-volatile alkali and a buffer salt by spreading said liquid on said surface in the form of a uniformly thin film, the quantity of the developing liquid contained in the film being substantially corresponding to that required to effect development of said surface. 120 125 130

6. The process for developing direct positive diazo prints which consists in saturating throughout its entire area the exposed surface of said prints with a developing liquid containing a non-volatile alkaline substance and a reducing agent non-decomposable by alkali by spreading said liquid on said surface in the form of a uniformly thin film, the quantity of the developing liquid contained in the film being substantially corresponding to that required to effect development of said surface. 70
7. The process according to claim 6 wherein the reducing agent is a thiosulphate. 75
8. The process for developing direct positive diazo prints which consists in saturating throughout its entire area the exposed surface of said prints with a developing liquid containing a non-volatile alkaline substance, an azo dyestuff component, and a reducing agent non-decomposable by alkali by spreading said liquid on said surface in the form of a uniformly thin film, the quantity of the developing liquid contained in the film being substantially corresponding to that required to effect development of said surface. 80
9. The process according to claim 8 wherein the reducing agent is thiosulphate. 85
10. The process for developing direct positive diazo prints which consists in saturating throughout its entire area the exposed surface of said prints with a developing liquid containing a non-volatile alkaline substance and a wetting agent by spreading said liquid on said surface in the form of a uniformly thin film, the quantity of the developing liquid contained in the film being substantially corresponding to that required to effect development of said surface. 90
11. The process for developing direct positive diazo prints containing a diazo compound of the type which can not be used together with azo-dyestuff components in the light sensitive layer which consists in saturating throughout its entire area the exposed surface of said prints with a developing liquid containing a non-volatile alkaline substance and an azo-dyestuff component by spreading said liquid on said surface in the form of a uniformly thin film, the quantity of the developing liquid contained in the film being substantially corresponding to that required to effect development of said surface. 95
12. The process for developing direct positive diazo prints containing a diazo compound of the type which can not be used together with azo-dyestuff components in the light sensitive layer which consists in saturating throughout its entire area the exposed surface of said prints with a developing liquid containing a non-volatile alkali, a buffer salt, and an azo-dyestuff component by spreading said liquid on said surface in the form of a uniformly thin film, the quantity of the developing liquid contained in the film being substantially corresponding to that required to effect development of said surface. 100
13. The process for developing direct positive diazo prints which consists in saturating throughout its entire area the exposed surface of said prints with a developing liquid containing a non-volatile alkaline substance by momentarily wetting the exposed surface with an excess of said liquid and removing the excess immediately thereafter, so as to depose a uniformly thin film of said liquid to said surface, the quantity of the developing liquid contained in the film being substantially corresponding to that required to effect development of said surface. 105
14. The process for developing direct positive diazo prints which consists in saturating throughout its entire area the exposed surface of said prints with a developing liquid containing a non-volatile alkali and a buffer salt by momentarily wetting the exposed surface with an excess of said developing liquid and removing the excess immediately thereafter, so as to depose a uniformly thin film of said liquid to said surface, the quantity of the developing liquid contained in the film being substantially corresponding to that required to effect development of said surface. 110
15. The process for developing direct positive diazo prints which consists in saturating throughout its entire area the exposed surface of said prints with a developing liquid containing a non-volatile alkaline substance and a reducing agent non-decomposable by alkali by momentarily wetting the exposed surface with an excess of said developing liquid and removing the excess immediately thereafter, so as to depose a uniformly thin film of said liquid to said surface, the quantity of the developing liquid contained in the film being substantially corresponding to that required to effect development of said surface. 115
16. The process for developing direct positive diazo prints which consists in saturating throughout its entire area the exposed surface of said prints with a developing liquid containing a non-volatile alkaline substance and an azodyestuff component by momentarily wetting the exposed surface with an excess of said developing liquid and removing the excess immediately thereafter, so as to depose a uniformly thin film of said liquid to said surface, the quantity of the developing liquid contained in the film being substantially corresponding to that required to effect development of said surface. 120
17. The process for developing direct positive diazo prints which consists in saturating throughout its entire area the exposed surface of said prints with a developing liquid containing a non-volatile alkali, a buffer salt and an azodyestuff component by momentarily wetting the exposed surface with an excess of said developing liquid and removing 125

ing the excess immediately thereafter, so as to depose a uniformly thin film of said liquid to said surface, the quantity of the developing liquid contained in the film being substantially corresponding to that required to effect development of said surface.

18. The process for developing direct positive diazo prints which consists in saturating throughout its entire area the exposed surface of said prints with a developing liquid containing a non-volatile alkaline substance, an azodyestuff component and a reducing agent non-decomposable by alkali by momentarily wetting the exposed surface with an excess of said developing liquid and removing the excess immediately thereafter, so as to depose a uniformly thin film of said liquid to said surface, the quantity of the developing liquid contained in the film being substantially corresponding to that required to effect development of said surface.

19. The process for developing direct positive diazo prints which consists in saturating throughout its entire area the exposed surface of said prints with a developing liquid containing a non-volatile alkaline substance, and a wetting agent by momentarily wetting the exposed surface with an excess of said developing liquid and removing the excess immediately thereafter, so as to depose a uniformly thin film of said liquid to said surface, the quantity of the developing liquid contained in the film being substantially corresponding to that required to effect development of said surface.

In testimony whereof we affix our signatures.

Dr. LODEWIJK PIETER FRANS van der GRINTEN.

Dr. KAREL JAN JOSEF van der GRINTEN.

ing the excess immediately thereafter, so as to deposite a uniformly thin film of said liquid to said surface, the quantity of the developing liquid contained in the film being substantially corresponding to that required to effect development of said surface.

18. The process for developing direct positive diazo prints which consists in saturating throughout its entire area the exposed surface of said prints with a developing liquid containing a non-volatile alkaline substance, an azodyestuff component and a reducing agent non-decomposable by alkali by momentarily wetting the exposed surface with an excess of said developing liquid and removing the excess immediately thereafter, so as to deposite a uniformly thin film of said liquid to said surface, the quantity of the developing liquid contained in the film being substantially corresponding to that required to effect development of said surface.

19. The process for developing direct positive diazo prints which consists in saturating throughout its entire area the exposed surface of said prints with a developing liquid containing a non-volatile alkaline substance, and a wetting agent by momentarily wetting the exposed surface with an excess of said developing liquid and removing the excess immediately thereafter, so as to deposite a uniformly thin film of said liquid to said surface, the quantity of the developing liquid contained in the film being substantially corresponding to that required to effect development of said surface.

In testimony whereof we affix our signatures.

Dr. LODEWIJK PIETER FRANS van der GRINTEN.

Dr. KAREL JAN JOSEF van der GRINTEN.

40

#### DISCLAIMER

1,841,653.—*Lodewijk Pieter Frans van der Grinten and Karel Jan Josef van der Grinten, Venlo, Netherlands. PROCESS FOR DEVELOPING POSITIVE DIAZO PRINTS.* Patent dated January 19, 1932. Disclaimer filed September 12, 1934, by the assignee, *Charles Bruning Company, Inc.*

Hereby enters its disclaimer of claims 7 and 9 of said patent.  
[Official Gazette October 9, 1934.]

51

55

60

65

## DISCLAIMER

1,841,653.—*Lodewijk Pieter Frans van der Grinten and Karel Jan Josef van der Grinten*, Venlo, Netherlands. PROCESS FOR DEVELOPING POSITIVE DIAZO PRINTS. Patent dated January 19, 1932. Disclaimer filed September 12, 1934, by the assignee, *Charles Bruning Company, Inc.*  
Hereby enters its disclaimer of claims 7 and 9 of said patent.  
[Official Gazette October 9, 1934.]